

## UNITED STATES PATENT OFFICE

2,449,806

## COLD HOBBABLE STEEL

Maurice C. Fetzer, Wyomissing, and William H. Kemper, Temple, Pa., assignors to The Carpenter Steel Company, Reading, Pa., a corporation of New Jersey

No Drawing. Application June 12, 1945.  
Serial No. 599,120

3 Claims. (Cl. 75—126)

1

This invention relates to alloy steels particularly adapted for making cold hopped articles.

An object of the invention is to produce alloy steels having unique combinations of properties including cold hobbability, low annealed hardness, ability to harden by both air cooling and oil quenching and in respect not only of the core but also of the case obtainable by case hardening, hot hardness of the core and the case, and stability of surface hardness of the case at temperatures up to about 1000° F., as well as toughness of the case and core when properly drawn and improved abrasion resistance particularly at high temperatures.

An alloy steel having the above mentioned combination of properties has particular value in the manufacture of cold hopped articles, e. g., molds and mold parts, for example, those used in the molding of plastics and plastic compositions requiring high molding temperatures; e. g., of the order of 500° F. to 800° F. Many of these compositions contain abrasive fillers which emphasize the need for a steel which will develop an abrasion resistant surface and will possess relative stability of surface hardness and abrasion resistance at relatively high molding temperatures.

There are available a number of irons and alloy steels which possess cold hobbability but are deficient in one or more of the above mentioned other properties. There are also a number of alloys which possess desirable degrees of hardness and ability to harden when air cooled or oil quenched as well as hot hardness, but are deficient in hobbability and therefore require that the mold cavity be machined. In other words, the experience in the art has been that the attainment of desirable properties such as high cold and hot hardness and ability to harden in air or oil is accompanied by lack of hobbability, and conversely that the property of hobbability is secured at the sacrifice of other desirable properties such as cold and hot hardness and ability to harden.

The advantages and objects of the invention will be further described as follows:

The steel alloys of this invention can be annealed to 125 maximum Brinell and therefore are easy to cold hop. After forming, the alloys can be hardened by heat treatment. Hardnesses of 25 to 43 R<sub>c</sub> are obtainable. The hardness referred to may be produced by air cooling without resorting to oil or water quenching although the alloys may be hardened by oil quenching. High strength accompanies the high hardness and persists at elevated temperatures and all of

the above properties are obtained without unduly sacrificing toughness. When carburized by known methods the alloys develop a case of normal depth which can be hardened to 60/66 R<sub>c</sub> by air cooling directly from the carburizing pack, thus eliminating the necessity of subsequent hardening treatment. The case also has better than ordinary resistance to corrosion, scaling and abrasion at elevated temperatures and the ability to retain its hardness at these temperatures. All of these properties of the carburized case are obtainable without unduly sacrificing toughness.

The invention will be defined in the claims and the principles thereof will be illustrated in Table I below by examples showing the analyses of certain preferred embodiments of the steel of the invention as follows:

Table I

| Examples   | 1                         | 2                         | 3                         | 4                         |
|------------|---------------------------|---------------------------|---------------------------|---------------------------|
| Carbon     | 0.05/0.15                 | 0.05/0.15                 | 0.05/0.15                 | 0.07/0.11                 |
| Manganese  | 0.10/1.00                 | 0.10/1.00                 | 0.10/1.00                 | 0.20/0.50                 |
| Silicon    | 0.10/0.25                 | 0.10/0.25                 | 0.10/0.25                 | 0.15/0.25                 |
| Chromium   | 4.75/6.00                 | 4.75/6.00                 | 4.75/6.00                 | 4.75/6.00                 |
| Molybdenum | 0.90/3.0                  | 0.90/3.0                  | 0.90/3.0                  | 0.90/1.30                 |
| or         |                           |                           |                           |                           |
| Tungsten   | 1.50/3.0                  | 1.50/3.0                  | 1.50/3.0                  | 1.50/3.0                  |
| Vanadium   |                           |                           | 0.20/0.50                 | 0.20/0.30                 |
| Cobalt     |                           |                           |                           |                           |
| Iron       | Substantially the balance | Substantially the balance | Substantially the balance | Substantially the balance |

The properties of the alloy steels produced in accordance with the above examples are shown in subjoined Table II.

Hobbability, one of the most important properties, is shown to some extent by the annealed Brinell hardness and to a more significant extent by what may be termed a hobbability index. This index is a measure of the depth of impression made in the metal by a hob  $\frac{1}{2}$ " in diameter under a load of 30 tons applied for 30 seconds after annealing (slow cooling) from 1600° F. and may be expressed in inches. The greater the depth in inches the more easily is the steel hopped.

A high heat treated core hardness is desirable because the core supports the case and prevents sinking. Where the steel is used without being carburized the high hardness is an index of the resistance to deformation and abrasion at the temperature of use.

In all the above examples the proportion of chromium may be 4 to 10 per cent instead of the narrower range shown without departing appreciably from the properties given in Table II.

Table II

[Numerical values are approximate]

|                                                                                                   | Example 1                          | Example 2                                 | Example 3                                 | Example 4                                 |
|---------------------------------------------------------------------------------------------------|------------------------------------|-------------------------------------------|-------------------------------------------|-------------------------------------------|
| Hobability Index As annealed from 1600° F.                                                        | 0.28                               | 0.27                                      | 0.30                                      | 0.30                                      |
| Annealed Hardness (Brinell) As slow cooled from 1600° F.                                          | 105-125                            | 105-125                                   | 105-125                                   | 125 max.                                  |
| Core Hardness—Oil Quenched from 1700°/1900° F.                                                    | 25-43 R <sub>c</sub>               | 25-43 R <sub>c</sub>                      | 25-43 R <sub>c</sub>                      | 38 R <sub>c</sub>                         |
| Core Hardness—Air Cooled from 1700°/1900° F.                                                      | 25-43 R <sub>c</sub>               | 25-43 R <sub>c</sub>                      | 25-43 R <sub>c</sub>                      | 38 R <sub>c</sub>                         |
| Case Hardness <sup>1</sup> Oil Quenched from 1700°/1900° F.                                       | 60-65 R <sub>c</sub>               | 60-65 R <sub>c</sub>                      | 60-65 R <sub>c</sub>                      | 64 R <sub>c</sub>                         |
| Case Hardness <sup>1</sup> Air Cooled from 1700°/1900° F.                                         | 60-65 R <sub>c</sub>               | 60-65 R <sub>c</sub>                      | 60-65 R <sub>c</sub>                      | 64 R <sub>c</sub>                         |
| Hot Hardness of core at 800° F.—Brinell after oil or air hardening from 1700°/1900° F.            | 325-360                            | 325-360                                   | 335-370                                   | 350                                       |
| Hardness of Case <sup>1</sup> after hardening from 1700°/1900° F. and drawing one hour at 800° F. | 50 R <sub>c</sub> (oil hardening). | 55 R <sub>c</sub> (oil or air hardening). | 57 R <sub>c</sub> (oil or air hardening). | 56 R <sub>c</sub> (oil or air hardening). |

<sup>1</sup> The carburizing treatment consisted of 6 hrs. at 1700° F. in a commercial carburizing compound.

The higher the case hardness at any given temperature the greater the resistance to wear, abrasion and indentation at that temperature.

The above table shows hardness values for the case as well as the core at ordinary or room temperatures after treating and also of the core at 800° F. The hot hardness of the case is indicated by the high hardness of the case after it has been drawn at 800° F.

It will be seen that all of the alloys of the above examples have in combination a number of desirable properties. The alloys of Example 2, containing molybdenum or tungsten, within the specified ranges, have distinct advantages over Example 1 in that they provide a high case hardness by air treating (air cooling) and therefore may be air treated directly from the pack. They also have a somewhat higher hot hardness of the case as indicated by the drawn hardness value of 55 R<sub>c</sub> as compared with 50 R<sub>c</sub> of the alloys of Example 1. The alloys of Examples 3 and 4 containing vanadium in the proportions specified have properties similar to those of Example 2 except that the drawn hardness is somewhat higher. Example 4 represents the preferred analysis.

All of the alloys are shown to have a high degree of hobbability notwithstanding the attainment of the other desirable properties. The addition of 1.5 to 2.5 per cent by weight of cobalt to any of the alloys of Examples 1 to 4 has the added advantage that the cobalt lowers the amount of carbon which is picked up during carburizing.

What is claimed is:

1. A cold hobbable steel containing carbon about 0.05 to 0.15 per cent, manganese about 0.10 to 1.00 per cent, silicon about 0.10 to 0.25 per cent, chromium about 4.00 to 10.00 per cent, vanadium up to 0.50 per cent, a metal selected from the group consisting of molybdenum and tungsten in the proportion of about 0.90 to 3.0 per cent molybdenum and about 1.5 to 3.0 per cent tungsten and the balance substantially iron, said steel having a Rockwell C hardness of about 25-43 when air cooled from 1700°-1900° F., a hot hardness of about 325-360 Brinell at 800° F., after air cooling from 1700°-1900° F., and when case hardened providing a case having a Rockwell C hardness of about 60-65 when air cooled from 1700°-1900° F.

2. A cold hobbable steel containing carbon about 0.05 to 0.15 per cent, manganese about 0.10

to 1.00 per cent, silicon about 0.10 to 0.25 per cent, chromium about 4.00 to 10.00 per cent, vanadium about 0.20 to 0.50 per cent and a metal selected from the group consisting of molybdenum and tungsten in the proportion of about 0.9 to 3.0 per cent molybdenum and about 1.5 to 3.0 per cent tungsten and the balance substantially iron, said steel having a Rockwell C hardness of about 25-43 when air cooled from 1700° F.-1900° F., a hot hardness of about 335 to 370 Brinell at 800° F. after air cooling from 1700°-1900° F. and when case hardened providing a case having a Rockwell C hardness of about 60-65 when air cooled from 1700°-1900° F. and about 57 when the hardened case is drawn at 800° F.

3. A cold hobbable steel containing carbon about 0.07 to 0.11 per cent, manganese about 0.20 to 0.50 per cent, silicon about 0.15 to 0.25 per cent, chromium about 4.00 to 10.00 per cent, vanadium about 0.20 to 0.30 per cent, about 0.90 to 1.30 per cent molybdenum and the balance substantially iron, said steel having a Rockwell C hardness of about 38 when air cooled from 1700° F.-1900° F., a hot hardness of about 350 Brinell at 800° F. after air cooling from 1700°-1900° F. and when case hardened providing a case having a Rockwell C hardness of about 64 when air cooled from 1700° F.-1900° F. and about 56 when the hardened case is drawn at 800° F.

MAURICE C. FETZER  
WILLIAM H. KEMPER

## REFERENCES CITED

50 The following references are of record in the file of this patent:

## UNITED STATES PATENTS

| Number    | Name          | Date          |
|-----------|---------------|---------------|
| 1,659,055 | Shimer et al. | Feb. 14, 1928 |
| 2,188,138 | Malcolm       | Jan. 23, 1940 |

## FOREIGN PATENTS

| Number  | Country       | Date           |
|---------|---------------|----------------|
| 338,556 | Italy         | Mar. 31, 1936  |
| 350,048 | Great Britain | June 11, 1931  |
| 472,464 | Great Britain | Sept. 16, 1937 |

## OTHER REFERENCES

65 Alloy Elements in Steel, pages 56, 66, and 67; Bain; published in 1939 by the American Society for Metals, Cleveland, Ohio.